

Jan. 19, 1965

D. W. RAHMES

3,166,465

BACKED PILE FABRIC AND METHOD OF PRODUCING THE SAME

Filed May 27, 1960



FIG. 1.



FIG. 3.



FIG. 2.



FIG. 4.

INVENTOR  
Donald W. Rahmes

BY

*Donald W. Rahmes*

ATTORNEY

1

3,166,465

## BACKED PILE FABRIC AND METHOD OF PRODUCING THE SAME

Donald W. Rahmes, Dover, Del., assignor to International Latex Corporation, Dover, Del., a corporation of Delaware

Filed May 27, 1960, Ser. No. 32,207  
14 Claims. (Cl. 161—66)

The present invention relates to improvements in textile fabrics and to a method for producing the same. More particularly, the invention relates to an improved composite structure as a backing for tufted loop or cut pile fabrics of the type used, for example, in floor and upholstery coverings.

The invention is described with particular reference to floor coverings of the tufted loop type, although it also provides improved backings for woven fabrics, either smooth surfaced or nap finished. Tufted carpeting is a composite structure in which the yarn forming the loops or cut pile in the carpet surface is needled through the interstices of a base fabric, such as burlap. The attachment of the legs or base segments of the yarn loops to the base fabric is made more permanent by coating the underside of the base fabric with a suitable binder or adhesive, referred to as a backing coat or back-size. In some instances, another separate and distinct lamina or component of the composite structure is added in the form of what may be called a secondary backing to impart a greater stiffness or dimensional stability to the floor covering. An example of a commercially used secondary backing is scrim, a woven fabric of large open mesh made of twisted paper strands. This must be secured to the base fabric by a separate procedure involving the spreading of an adhesive coat and laying of the scrim onto the base fabric after the backing coat has been applied. The scrim is thus a lamina separate from the backing coat on the base fabric.

The present invention advantageously provides an improved backing characterized by a more compact composite structure, imparting increased dimensional stability to the fabric in all directions, and a flexible backing coat which is reinforced with a fibrous web. The reinforced backing coat maintains its flexibility and resists cracking with advantageously high loadings of filler in the coating composition.

The invention accordingly is characterized by an article of manufacture comprising a tufted loop or pile fabric having a preformed woven base material in which the tufts are inserted, and a supporting lamina adhered to the underside of said base fabric comprising a coating of binder material, and a web of fibers disposed in the coating layer and reinforcing the same. The binder material coats the fibers of the web and permeates and penetrates the interstices thereof, thereby securing the base segments of the tufts to said base fabric, as well as bonding the web to both the base segments of the tufts and the base fabric.

The invention also provides the advantage that the improved fabrics of the invention are made by a method which requires only a single application of the backing compound, which acts as an adhesive for accomplishing this multiple bonding.

Thus, the improved textile product is produced by a method which is relatively simple compared to the slower two step process when scrim is utilized as a secondary backing for tufted carpets.

By the method of the present invention, a thin web of fibers, for example, carpet rayon (acetate or viscose) fibers, preferably lightly bonded, is laid on the underside of the woven base fabric of a tufted carpet. A flowable or liquid binding agent, for example, rubber latex, is

2

used to impregnate the fibrous web such that it coats the fibers and penetrates through the web thereby coating the base loops of the tufts and the underside of the base fabric. Thereafter the coated laminated material is subjected to drying, and to curing conditions, if necessary, to solidify the binder thereby forming a secure bond between the base loops of the tufts and the base fabric, and forming a lamina which is a fiber-reinforced backing coat. Alternatively, the latex coating may be applied to the underside of the base fabric and the reinforcing web pressed into the flowable coating to form the fiber reinforced backing lamina.

The invention is described in greater detail with reference to the accompanying drawings which illustrate particular embodiments thereof and are not intended to constitute a limitation thereon, in which:

FIGURE 1 is an enlarged schematic illustration of a so-called tufted carpet structure,

FIGURE 2 is a schematic view of a method for producing the articles of the invention, and

FIGURE 3 is a schematic view of an alternative method where the carpet is coated with a backing compound and the fibrous web is pressed into the coating to form the backing lamina.

FIGURE 4 is an exploded view of the composite structure showing the various components and reinforced backing coat in greater detail.

Referring to FIGURES 1 and 4, a pile fabric 10 having the composite structure of the invention is shown in which the loops 1 are shown in an exaggerated size in the position in which they are needled through a woven burlap base fabric 2. The base loops or segments 3 are formed by the needling of the pile yarn through the base fabric interstices to the underside 4 of the base fabric 2. The base loops 3 are bonded to the base fabric by means of adhesive binder portions 5 which have penetrated through the support lamina 20. The support lamina 20 is made up essentially of two components, a web of fibers 6 embedded in a matrix 7 of solidified binder.

The binder material may be an aqueous dispersion, a solution, or other suitably liquid or flowable preparation, including hot melts in case of thermoplastic binders where the melting temperatures are below those which would be injurious to the fabric.

For most applications of the invention the binder should be flexible and resilient. Preferably it is an aqueous dispersion of an elastomeric material, such as latices of natural and synthetic rubber. The latex may be foamed, or in some cases merely agitated, to produce more loft and a cellular structure in the support lamina. Any of the known elastomers are suitable for this purpose including natural rubber, synthetic polyisoprene, butadiene-styrene, butadiene-acrylonitrile, chloroprene, polyisobutylene and other types of rubbery binders. Where flexibility without elasticity will suffice, thermoplastic binders of a suitable type may be used, such as polyvinyl chloride, polyvinyl acetate, acrylate resins, and acrylate-vinyl copolymers, and other vinyl copolymers; all of which are well known and which of themselves form no part of the invention. Mixtures of elastomers and resins may be employed as a backing coat or binder and particularly minor quantities of thermoplastic resin solids and a major quantity of vulcanizable elastomer.

Referring to FIGURE 2, a method of producing the articles of the invention is illustrated in which the fibrous web 6, which may be formed on conventional carding or garnetting machines, or which may be air deposited for more random distribution of fibers, is fed from roll 21 above the conveyor 22 upon which the pile fabric 10 is conveyed in an inverted position with the base fabric 2 exposed. The web 6 is superimposed on the pile fabric 10 in contact with the underside 4 of the base fabric 2 by

means of feed and combining roll 25. The web superimposed on the fabric 10 is coated at 26 with a flowable binding material, such as a vulcanizable rubber dispersion or latex fed through hose 27, and the coated composite is passed beneath a doctor blade or roll 28 so that the fibers in the web 6 are coated and the web saturated with the liquid binder. The binder penetrates through the loose web to coat the base loops 3 of the pile fabric and the underside of base fabric 2.

In FIGURE 3, the underside 4 of base fabric 2 of the carpet is first coated with a layer 8 of binder, e.g., rubber latex in the same manner as shown at 26 in FIGURE 2. The fibrous web 6 is then pressed into the wet coating on the base fabric by combining roll 25. The latex coating penetrates the web, and the coating and web are united into a single lamina secured to the base fabric 2 and the base loops 3 of the pile fabric 10. The coated lamina is then passed through a drying and curing oven (not shown) where the binder is solidified and cured to provide the supporting or reinforcing lamina 20 made up of the reinforcing fibrous web 6 coated and bonded with the solid binder 7. This lamina is strongly secured to the base fabric by the binder portions which penetrate into the web and which remain integral with the binder portions permeating the web. The supporting lamina is also strongly bonded to the base loops 3 of the pile fabric on the underside of the base fabric, and the loops 3 are more tightly secured to the base fabric 2. This in turn strengthens the entire structure against slipping or pulling out of the filaments forming the loops or pile, and greatly increases dimensional stability.

The fleece or web of fibers contained or embedded in the binder coating reinforces the coating. This permits utilization of greater quantities of fillers, extenders or loading agents in the binder dispersion without excessive cracking or other deterioration of the coating. This reinforcement of the coating and greater dimensional stability in the structure of the composite are advantages not limited to unwoven or tufted carpets, and therefore the invention is fully applicable to woven carpeting and other woven pile fabrics.

The flexibility or stiffness of the composite may desirably be varied not only by the choice of binder, but also by variations in the thickness of non-woven fibrous web. Also its density, weight and fiber composition may be varied to provide the composite structure with desired "hand," appearance, resilience, and flexibility. The composite may be made lighter in weight and of improved dimensional stability, even with increased loading of the binding agent, compared to scrim or reticulate lamina adhesively secured to the base fabric.

The fibrous material may be batts or webs of a plurality of layers or cards or oriented or randomly disposed fibers made on suitable dry web-forming means, such as conventional carding or garnetting machines, or air deposited. The web may also be water-laid on wet-web forming devices, e.g., Fourdrinier machines. The webs may be made of multi- or mono-filamentary materials, i.e., yarns or threads of animal or vegetable fibers, such as wool, hair, cotton, flax, sisal, hemp, and other naturally occurring cellulosic or proteinaceous fibers, or synthetic fibers, such as rayon, viscose or acetate, nylon, polyester, polyurethane, acrylics and other fiber-forming thermoplastic polymers and mixtures of such fibers. Inclusion of jute or other hard fibers which have hairs or fibrilles protruding from the main strands is particularly desirable. This provides a nap-like or fibrous finish to the backing. The fibrous web may even consist of felted fibers or webs, such as paper or tissue from cellulosic pulps, provided that the web or felt is of sufficiently a porous open structure or network to permit penetration by the binder and embedding of the web in the binder after the latter is solidified. Flock or loose fibers may be used in place of a preformed web, where the flock or loose fibers are co-deposited to provide a fiber-reinforced binder layer or coating.

The web is preferably prebonded with any binder such as those mentioned above. This is simply to permit handling in subsequent operations and spot bonding or very small binder contents of only 5-10% are sufficient.

The length and diameter of the fibers making up the web may be widely varied whiel obtaining the advantages of the invention. Fiber lengths of above one-half inch to below two inches at present have given best results in terms of avoiding cracking of the coating at increased loading in the binder, and "hand" or appearance. The fiber diameters which at present appear particularly advantageous are from about 10 to 40 denier. It is to be understood, however, that even paper pulp fibers of much shorter length than one-half inch and other fibers of diameter, e.g., 3-5 denier are usable with a lesser increase in improved properties in the composite.

The webs may also vary in weight or density, such as from below one up to several ounces per yard. It has been found that the best reinforcing properties in the binder-web lamina are found when the thickness of the web is at least equal to the thickness of the coating of binder. When this condition is observed the material exhibits a much resistance to cracking of the binder layer upon bending and flexing of the composite fabric, even at very high loading of the binder compared to a backing coat without the reinforcing web.

The invention is further illustrated by reference to the following example which is intended to provide a complete specific embodiment of the invention.

A fibrous web consisting of carpet rayon fibers of 17 denier per filament and having a weight of approximately two ounces per square yard was laid on the underside of a jute burlap base fabric of a tufted carpet of a blend of wool and rayon yarns in the manner above-described in connection with FIGURE 2. A quantity of carpet backing latex compound having the composition given below and with a conventional sulfur curing system including accelerator was poured on the laminated material and the coating was uniformly spread across the surface of the web and pressed into the same by means of a doctor blade. This procedure caused the liquid latex to penetrate the web and wet the base loops of the pile fabric and the underside of the backing, as well as substantially filling in the interstices of the fibers in the web and thoroughly coating the fibers. A strong and flexible composite pile fabric was obtained by drying and curing the binder under conventional conditions, for example, heating at 250° to 300° F. for 15 to 30 minutes. Samples of the fabric with the web reinforced backing coat were subjected to repeated 180° (zero thickness) bending, and even when the bent sample was twisted, cracking of the backing coat did not occur.

#### Latex coating compound composition

| Constituents                                           | Parts (Dry Weight) |
|--------------------------------------------------------|--------------------|
| Butadiene-styrene latex                                | 100.               |
| Sulfur Cure System:                                    |                    |
| 2 parts sulfur                                         |                    |
| 5 parts ZnO                                            |                    |
| 2 parts Ethyl Zimate                                   |                    |
| 1 part Zemite special (mercaptobenzothiazole)          | 10 Total.          |
| Casein                                                 | 2.                 |
| Potassium oleate soap                                  | 2.                 |
| Agarite Superlite (antioxidant)                        | 1.                 |
| Whiting (loading or extender)                          | 290/300 total      |
| Titanium dioxide (TiO <sub>2</sub> ) (pigment loading) | 10/ loading.       |

The procedure of the above example was repeated with omission of the fibrous web of rayon fibers. The unreinforced coating cracked badly with the same 300 parts loading per 100 parts dry rubber in the latex compound upon mere bending without twisting. Suitable commercial carpet backing latex compounds for carpets of this type contain no more than 300 parts of loading, and generally less for proper strength of bond.

Other samples of web-reinforced backings were made

up from paper pulp fibers of a mean diameter of 3 denier and a mean length of 0.25 inch. Even these samples did not fail on bending the fabric as did those with unreinforced coatings with equal loading (300 parts).

Samples were prepared using 17 denier acetate fibers of mean length of  $1\frac{1}{16}$  inches, and the loading in the latex binder compound was varied from 300 parts to 1000 parts. Even at 1000 parts loading there was no cracking of the backing on bending those samples in which the latex coating layer did not exceed the web thickness. Loadings of 1000 parts, however, are not generally recommended because the binder solids in the coating are then highly extended. Where the coating layer was heavier and exceeded the thickness of the web, cracking on bending was more pronounced even at 400 to 500 parts loading.

Samples prepared with the same tufted carpet and latex backing compound using scrim as a secondary backing were heavier and more costly, lacked desired dimensional stability on diagonal pull, and lacked desirable hand compared to the samples having the improved composite structure of this invention. In addition, the appearance of the underside of carpet samples with the backing of the invention is far superior, i.e., less coarse and neater than that of scrim-backed samples. The fibrous web-reinforced latex backing coat is applicable to any fabrics for floors, walls, deck, panel, and furniture coverings, where increased hand and elimination of coating failure with loading are desired.

Various changes and modifications may be made within the scope of my invention, and the specific embodiments above-described and shown in the accompanying drawings should be regarded as illustrative only and not as a limitation on the scope of the appended claims.

What I claim:

1. An article comprising a composite textile having a finished upper surface of filamentary material, said material having base portions held in a base fabric, a non-woven fibrous web contacting said base portions, and a mass of binder coating the fibers of said web and permeating and penetrating the interstices thereof to unite the web to said base portions and to substantially completely embed said web in a binder matrix.

2. A pile fabric with tufts held in a woven base fabric, a non-woven fibrous web engaging the underside of said base fabric, and a mass of aqueous dispersion-deposited flexible binder coating the fibers of said web and permeating the interstices thereof, said mass of binder uniting the web to said base fabric and to the base of the tufts, and forming with the fibrous web a resilient backing lamina in which the web extends throughout the thickness of the mass of binder.

3. A floor covering having a tufted surface of filamentary material with base segments thereof inserted through a woven base fabric, a non-woven fibrous web contacting the base segments of the filaments, and a mass of flexible rubbery binder coating the fibers of said web and permeating the interstices thereof to form a fibrous web-reinforced backing coat in which the web extends throughout the thickness of the mass of binder, and a portion of said binder coating the base fabric and the base segments of the tufted filaments and uniting the web thereto and to the base fabric.

4. A floor covering according to claim 3 in which the rubbery binder is deposited from latex.

5. A woven carpet fabric having a pile surface interwoven with a base fabric, a non-woven fibrous web contacting the underside of said base fabric, and a mass of

flexible rubbery binder coated on the fibers of said web and uniting it to said basic fabric, said mass of binder forming with said web a resilient backing lamina in which the web is substantially completely embedded in said binder.

5 6. A woven carpet fabric according to claim 5 in which the binder is latex rubber.

7. A method of producing a composite pile fabric structure, which comprises placing a non-woven fibrous web in contact with the underside of the base material of said pile fabric, applying a flowable binder material to said web to coat the fibers and permeate the interstices thereof, the binder penetrating to the base fabric thereby bonding the web to said base fabric and forming with the web a fiber-reinforced resilient backing lamina in which the web is substantially completely embedded in said binder.

10 15 8. A method according to claim 7 in which the binder is coated in aqueous dispersion form and the composite is dried.

10 20 9. A method according to claim 8 in which the binder is a rubber latex and after coating of the web, the composite is dried and the rubber is cured.

10 25 30 35 10. A method of producing a composite floor covering having a tufted surface of filamentary material with base segments inserted through a woven base fabric, which comprises placing a web of non-woven fibers in contact with said base segments, applying a flowable elastomeric binder to the web to coat the fibers of the web, and by penetration through the web also to coat the base segments of the filamentary material and the underside of the base fabric, and solidifying said binder thereby bonding the web, the segments, and the base fabric into a resilient laminated structure having a fiber-reinforced flexible backing lamina of elastomeric binder in which the web extends throughout the thickness of said binder.

10 35 11. A method according to claim 10 in which the binder is coated an aqueous dispersion form and the coated composite is dried.

10 40 12. A method according to claim 11 in which the binder is a rubber latex and after coating of the web, the composite is dried and the rubber is cured.

10 45 13. A method of producing a composite pile fabric, which comprises depositing a layer of flowable binder material on the underside of the base of said pile fabric, and combining with said layer a web of non-woven fibrous material to form a fiber-reinforced binder lamina secured to said base, the web in said lamina extending throughout the thickness of the layer of binder.

10 50 14. A method according to claim 13 in which the base fabric is coated with a layer of latex, and the fibrous web is fully integrated into said latex layer to form a single fiber-reinforced flexible lamina.

References Cited in the file of this patent

55 UNITED STATES PATENTS

|           |                 |               |
|-----------|-----------------|---------------|
| 1,918,849 | Larson          | July 18, 1933 |
| 2,266,846 | Buff            | Dec. 23, 1941 |
| 2,512,727 | Rice            | June 27, 1950 |
| 2,550,686 | Goldman         | May 1, 1951   |
| 2,675,337 | Walker et al.   | Apr. 13, 1954 |
| 2,752,277 | Keen            | June 26, 1956 |
| 2,787,571 | Miller          | Apr. 2, 1957  |
| 2,948,650 | Jackson         | Aug. 9, 1960  |
| 3,007,836 | McNamara et al. | Nov. 7, 1961  |
| 3,060,072 | Parlin et al.   | Oct. 23, 1962 |